

# UNITED STATES PATENT OFFICE.

FREDERICK M. BECKET, OF NIAGARA FALLS, NEW YORK, ASSIGNOR TO ELECTRO METALLURGICAL COMPANY, A CORPORATION OF WEST VIRGINIA.

## PROCESS OF REDUCING METALLIC OXIDS.

No. 854,018.

Specification of Letters Patent.

Patented May 21, 1907.

Application filed September 23, 1905. Serial No. 279,857.

*To all whom it may concern.*

Be it known that I, FREDERICK M. BECKET, a subject of the King of Great Britain, residing at Niagara Falls, in the county of Niagara and State of New York, have invented certain new and useful Improvements in Processes of Reducing Metallic Oxids, of which the following is a specification.

This invention is a process for the production of metals and alloys of low silicon and carbon content, and is more particularly applicable to the metals chromium, tungsten, molybdenum and vanadium and to the alloys of these metals with iron or nickel.

15 The invention consists in reducing a suitable oxid or oxygen-containing compound or mixture of oxids by silicon, the silicon being used in proportions and under conditions to insure a low silicon content of the product. 20 The conditions necessary for substantially complete reduction of the refractory metallic oxid or oxids above mentioned and the production of metals or alloys of low silicon and carbon content are obtainable so far as known 25 only in an electric furnace. Preferably a basic flux is used to combine with the silica derived from the oxidation of the silicon.

Metallurgists have long been familiar with the reducing action of silicon on certain metallic oxids, such as oxid of iron, and advantage is taken of this chemical reaction in many industries,—for example in the manufacture of steel. In these cases the silicon exists in the form of an alloy, its reducing 35 properties are employed as a means of eliminating it from the finished product rather than as a means of producing further quantities of metal, and the proportion of reducible oxid used for its removal is largely in excess of that theoretically necessary. In the 40 form of metallic silicides, silicon is employed to reduce metallic oxids dissolved in molten metals, and in this form it is also used for the production of double silicides of the metals, 45 and of alloys containing considerable proportions of silicon. Until a comparatively recent date metallic silicon has not been considered an article of commerce. The metal is now produced in the electric furnace, often 50 associated with considerable quantities of iron, at such cost and in such quantity as to permit its economical application as a reducing agent in certain electro-metallurgical operations.

I have found that silicon, although not so 55 electro-positive as aluminium, may be advantageously employed in the electric furnace as a reducing agent in the production of chromium, molybdenum, tungsten and vanadium, or the iron or nickel alloys of these 60 metals. When a suitable mixture consisting of silicon, an oxid of one or more of the above metals, and a basic flux is treated in an electric furnace, the advantages of a continuous and very rapid process may be obtained, and 65 by suitably proportioning the ingredients of the charge the silicon content in the reduced metals may be made as small as 0.01 percent. or less.

As a specific example of the process I will 70 describe its application to the manufacture of low carbon and low silicon ferrochromium from chromite. As the chromium in chromite exists as chromium sesquioxid,  $\text{Cr}_2\text{O}_3$ , and practically all the iron as ferrous oxid, 75  $\text{FeO}$ , the following reactions take place.



A fair commercial grade of chromite contains 52 percent.  $\text{Cr}_2\text{O}_3$  and 16 percent.  $\text{FeO}$ , and 100 pounds of this ore will therefore require, according to the above reactions, 17.7 pounds silicon for complete reduction of the chromium and iron. A representative analysis of ferrochromium made by this method is as follows: Chromium 71.00 percent.; iron 28.40 percent.; carbon 0.50 percent.; silicon 0.10 percent.

It is advantageous to use the silicon in a 90 fairly fine state of division and the metal is generally crushed so that it will all pass a ten-mesh screen. However, the state of division of the silicon depends on the scale of the operation. The use of a basic flux in the 95 production of ferrochromium is not essential although advantageous. Most commercial chromites contain from 8 to 15 percent.  $\text{Al}_2\text{O}_3$  and 8 to 15 percent.  $\text{MgO}$ . These materials serve as basic flux for the silica present in the 100 ore and for that produced by oxidation of the silicon; but the proportions are such that to maintain this slag fluid for tapping, a higher temperature is necessary than that required for complete reduction of the chromium and 105 iron oxids by silicon.

By mixing chromite and silicon in practically theoretical proportions, together with

some basic flux such as lime, and bringing the mixture to a state of fusion in an electric furnace, a very high yield of chromium and iron may be obtained from the ore used and the alloy contains only fractions of a percent. of carbon and silicon. It is not essential that the proportions be precisely those indicated by theory, because in the case in which very low silicon content is required in the alloy, (less than 0.2 percent.), the chromite is used in very slight excess of the theoretical proportions; and in the case in which a silicon content as high as one percent. may be permitted, the silicon is used in very slight excess. There is a slight advantage in the latter method on account of the fact that the yield of metal from the ore is slightly higher. In both cases, however, the variations from the theoretical proportions are small and the yields high.

I do not limit myself to any particular type of electric furnace but I have found it advantageous to carry on the reduction continuously in an electric furnace in which the current passes through a molten bath of a mixture of ore, silicon and flux, and from which part or all of the metal or slag may be withdrawn as desired. It is possible to melt a mixture of silicon and oxid or oxygen containing compound of the metals referred to and not effect complete reduction; and to obtain a high yield of the desired metal or alloy and to insure a low silicon content therein, I have found it advantageous to feed the mixture to a bath which is constantly maintained at a temperature higher than that necessary to cause some reaction.

The electric furnace operation may be carried out by fusing the ore and flux and then adding thereto the metallic silicon, or by fusing a mixture of ore and silicon and adding flux to this bath from time to time, but I have not found these methods to be as efficient as that above described.

As the reaction between silicon and the above mentioned metallic oxides is strongly exothermic, a relatively small amount of electrical energy is required for the reduction; moreover the reaction proceeds without evolution of gas which is of great practical advantage. The use of silicon as a reducing agent is highly advantageous in practice as compared with the use of aluminium for several reasons, among which may be mentioned the relatively large weight of metal which is separated per unit weight of the reducing agent; the comparative ease with which silicon is obtained in a fine state of division whereby a more intimate mixture is obtainable; the fact that with such mixtures the reaction proceeds more quietly and with less loss of material; and more particularly because silicious ores, which are relatively inexpensive, may be successfully used. Aluminium reduces silicon from the silica in-

variably present in such ores as chromite, wolframite, etc., and I have found in practice that silicon so reduced, as well as portions of the aluminium fused for reduction, alloy with the reduced metal, thereby necessitating either a costly selection of ores or other expensive method in case a product low in silicon is required. Furthermore in such case there is liability to the introduction of both silicon and aluminium into the metal, and in practice it is found to be more difficult to eliminate small percentages of the latter metal than of the former.

By the expression "refractory metallic oxids", occurring in certain claims, I mean such metallic oxids as require for their reduction by silicon the application of heat to the charge to maintain a reacting temperature, the reaction not being of a self-propagating character.

I claim:

1. The process of reducing refractory metallic oxids which consists in smelting a charge containing a metallic oxid reducible by silicon and silicon, the silicon being present in substantially the proportion required to combine with the oxygen of said oxid whereby a substantially complete oxidation of the silicon is secured and a product low in silicon is obtained, substantially as described.

2. The process of reducing metallic oxids which consists in electrically smelting a charge containing a metallic oxid reducible by silicon and silicon, the silicon being present in substantially the proportion required to combine with the oxygen of said oxid whereby a substantially complete oxidation of the silicon is secured and a product low in silicon is obtained, substantially as described.

3. The process of reducing refractory metallic oxids which consists in smelting a charge containing a metallic oxid reducible by silicon, silicon and a basic flux, the silicon being present in substantially the proportion required to combine with the oxygen of said oxid whereby a product low in silicon is obtained, substantially as described.

4. The process of reducing metallic oxids which consists in electrically smelting a charge containing a metallic oxid, reducible by silicon silicon and a basic flux, the silicon being present in substantially the proportion required to combine with the oxygen of said oxid whereby a product low in silicon is obtained, substantially as described.

5. The process of reducing metallic oxids which consists in passing an electric current through a molten bath containing a metallic oxid reducible by silicon and silicon, the silicon being present in substantially the proportion required to combine with the oxygen of said oxid whereby a product low in silicon is obtained, substantially as described.

6. The process of reducing metallic oxids which consists in passing an electric current

through a molten bath containing a metallic 5  
oxid, reducible by silicon silicon and a basic  
flux, the silicon being present in substantially  
the proportion required to combine with the  
oxygen of said oxid whereby a product low in  
silicon is obtained, substantially as described.

7. The continuous process of reducing me-  
tallic oxides which consists in passing an elec-  
tric current through a molten bath contain-  
ing a metallic oxid, reducible by silicon sili-

con and a basic flux, adding fresh portions of  
the charge and withdrawing the products as  
required, substantially as described.

In testimony whereof, I affix my signature  
in presence of two witnesses.

FREDERICK M. BECKET.

Witnesses:

JAS. M. WHITING,

WM. L. HEIM.